

Dec. 26, 1944.

C. R. HORWEDEL

2,365,959

STAINLESS STEEL WIRE

Filed Sept. 26, 1941

Fig. 1.



TRANSPARENT WAX FILM DIE-WORKED  
INTO WIRE SURFACE TO RENDER IT  
SUBSTANTIALLY INVISIBLE.

Fig. 2.



COILED STAINLESS STEEL WIRE  
STOCK SHOWN IN FIG. 1.

INVENTOR

CHARLES RICHARD HORWEDEL,  
by: *John E. Jackson*  
his Attorney.

Patented Dec. 26, 1944

2,365,959

# UNITED STATES PATENT OFFICE

2,365,959

## STAINLESS STEEL WIRE

Charles Richard Horwedel, Lakewood, Ohio, assignor to The American Steel and Wire Company of New Jersey, a corporation of New Jersey

Application September 26, 1941, Serial No. 412,509

1 Claim. (Cl. 29—180)

This invention relates to stainless steel wire, the object being to provide this product in such a form that it can be subjected to cold-forming operations with less of a tendency for its surface to be marred or scratched, and so that it can be more easily coiled and uncoiled.

The present application is a continuation, in part, of a copending application filed by the same inventor on May 21, 1940, and bearing Serial No. 336,441. This application has now issued as Patent No. 2,260,455.

Stainless steel wire is produced by drawing stainless steel through dies, this imparting a highly finished surface which, in practically all instances, it is desirable to maintain. Due to its analysis, the wire is inherently very hard so that it strongly resists cold deformation, this resulting in high die pressures during the production of the wire, and necessitating the use of high pressures when this wire is ultimately cold-formed into articles of commerce. For instance, stainless steel wire of relatively high carbon content, such as .14% carbon, is used to make brushes, springs, wire ropes, etc., the fabrication of which requires cold deformation of the wire beyond its elastic limit so as to set it in the form of the product desired, and this, in turn, is done by automatic machinery using fixed guides, and the like, past which the wire is forced and which deflect the wire so as to set it in its desired form. In all such instances, a problem is encountered in that, due to high pressures between the moving wire and the fixed guide parts, there is a decided tendency for the wire to become marred or scratched, this being disadvantageous for various reasons, such as the lowering of fatigue life caused by a scratch in the case of a spring, the acceleration of corrosion resulting from such a defect in the case of all products, and the general detraction from the appearance in the case of those products which are required to have eye-appeal.

In the copending application, the problems encountered in the drawing of such wire are disclosed as being solved by continuously drawing stainless steel wire through a series of dies of the required hardness, the wire being coated with a solid wax and drawn successively through the dies, the wax melting as the wire draws through each die and being then immediately bathed with a fluid coolant so as to resolidify the wax so that it is solid when the wire encounters a succeeding die. It is disclosed that the wax must have a melting temperature of not less than 40° C., and that it must, in each instance, be bathed by the coolant upon leaving each die, including the last die, so that the wire retains a waxed coating. This wax coating remains on

the finished product and facilitates its further processing or manipulation.

The wax used may be beeswax, Chinese wax, paraffin, bayberry wax, or carnauba wax, all having a melting temperature exceeding 40° C. Due to the drawing operation, this wax is worked into the surface of the stainless steel wire under exceedingly high pressure and provides a markedly improved product.

10 The product that results from this new method, carries a wax film covering its surface that is worked into this surface under high pressure, as is mentioned above, the film being substantially invisible but giving the wire a waxy feel and facilitating its coiling and uncoiling. Although substantially invisible, this wax film provides a lubricating effect preventing marring of the highly finished surface of the stainless steel wire when it is forced past fixed parts during its fabrication into cold-formed articles, such as springs, brushes, wire rope, etc.

In addition to the above advantages, stainless steel wire has the characteristics that when it is coiled or uncoiled the various convolutions tend to stick together due to their having such a high coefficient of friction, and although the wire with its wax film looks just like the prior art stainless steel wire, it will be found to handle much easier in such instances. Furthermore, there is much less chance of the surface of this product being marred during shipping, when it carries the wax film disclosed herein. It is to be understood that in all instances the wax film may be easily removed from the fabricated articles should this prove desirable, although in most instances it is unnecessary. All of the waxes mentioned may be removed by various solvents, carbon tetrachloride having been found satisfactory.

25 30 35 40 45 The wire disclosed herein is illustrated by the accompanying drawing, Figure 1 being a greatly enlarged cross-section of the wire showing the wax film, while Figure 2 shows in elevation a coil of the wire shown by Figure 1.

I claim:

50 55 Stainless steel wire in coil form with its surface carrying a compressed film consisting solely of wax of the class consisting of beeswax, Chinese wax, paraffin, bayberry wax and carnauba wax having melting temperatures exceeding 40° C., said film being die-worked into the surface of the wire under pressure so extremely high that the wire is reduced in size by the die-working, said film being substantially invisible while being detectable by the wire having a waxy feel giving it antifriction properties.

CHARLES RICHARD HORWEDEL.